

## UNITED STATES PATENT OFFICE.

SIGISMUND FUCHS, OF HOCHST-ON-THE-MAIN, GERMANY, ASSIGNOR TO I. G. FAR-BENINDUSTRIE AKTIENGESELLSCHAFT, OF FRANKFORT-ON-THE-MAIN, GERMANY, A CORPORATION OF GERMANY.

PROCESS FOR PRODUCING A PREPARATION FOR SOFTENING AND OILING TEXTILE FIBERS.

No Drawing. Application filed March 24, 1927, Serial No. 178,139, and in Germany March 27, 1926.

The present invention relates to the manufacture of a softening and oiling preparation to be used in the spinning of textile fibers.

5 Softening and oiling preparations to be used in the spinning of textile fibers are generally produced by emulsifying olein and water with an alkali, ammonia or sodium carbonate added thereto, whereby the olein 10 becomes partly saponified.

Now I have found that in the manufacture of softening and oiling preparations for use in spinning there may be obtained emulsions of an extraordinary stability by simultaneously adding to the mixture of an oil and water alkylated cellulose and sulfonic acids or water-soluble salts of such aromatic or hydrated aromatic sulfonic acids as contain as side chain hydrocarbon residues such 20 as the alkyl-, aryl-, aralkyl-, or cycloalkyl residue, either alone or mixed one with another. The oiling preparation thus produced possesses above all the advantage that it has not only an excellent emulsifying 25 power, but also a great wetting power, which ensures a rapid and uniform impregnation of the wool fibers with the softening liquid. Furthermore, the oiling preparation thus obtained has no tendency to gelatinize, a fact 30 which is of the highest importance for its practical use.

The oiling preparation may be produced with or without the addition of an alkali. The wool fiber is preferably moistened by 35 means of one of the usual spraying devices.

The following example serves to illustrate my invention, but is not intended to limit it thereto, the parts being parts by weight.

300 parts of water are mixed with an aqueous solution of 2, 5 parts of dimethyl cellulose and 2, 5 parts of sodium isopropyl-naphthalenesulfonate. Into this mixture are run, while continuously stirring, 80 parts of olein, until the latter forms an entirely 40 homogeneous emulsion. The oiling preparation so obtained is then applied in the usual manner.

Instead of sodium isopropylnaphthalene-sulfonate there may also be used for instance 45 sodium dibutylnaphthalenesulfonate, sodium

benzylnaphthalenesulfonate, butylnaphthalene sulfonic acid, whereas instead of olein there may be used olive oil, a mineral oil or the like, or mixtures of these oils.

I claim:

1. The process for producing a preparation for softening and oiling textile fibers, which consists in adding to the mixture of an oil and water as an emulsifying agent an alkylated cellulose together with a water-soluble aromatic sulfonic acid compound containing a hydrocarbon residue as side chain. 55

2. The process for producing a preparation for softening and oiling textile fibers, which consists in adding to the mixture of an oil and water as an emulsifying agent an alkylated cellulose together with a water-soluble hydrated aromatic sulfonic acid compound containing a hydrocarbon residue as side chain. 60

3. The process for producing a preparation for softening and oiling textile fibers, which consists in adding to the mixture of an oil and water as an emulsifying agent an alkylated cellulose together with a water-soluble salt of an aromatic sulfonic acid containing a hydrocarbon residue as side chain. 65

4. The process for producing a preparation for softening and oiling textile fibers, which consists in adding to the mixture of an oil and water as an emulsifying agent an alkylated cellulose together with a water-soluble salt of a hydrated aromatic sulfonic acid containing a hydrocarbon residue as side chain. 80

5. The process for producing a preparation for softening and oiling textile fibers, which consists in adding to the mixture of an oil and water as an emulsifying agent an alkylated cellulose together with a water-soluble aromatic sulfonic acid compound containing several hydrocarbon residues as side chains. 90

6. The process for producing a preparation for softening and oiling textile fibers, which consists in adding to the mixture of an oil and water as an emulsifying agent an alkylated cellulose together with a water-soluble hydrated aromatic sulfonic acid 100

compound containing several hydrocarbon residues as side chains.

7. The process for producing a preparation for softening and oiling textile fibers, which consists in adding to the mixture of an oil and water as an emulsifying agent an alkylated cellulose together with a water-soluble salt of an aromatic sulfonic acid containing several hydrocarbon residues as side chains.

8. The process for producing a preparation for softening and oiling textile fibers, which consists in adding to the mixture of an oil and water as an emulsifying agent an alkylated cellulose together with a water-soluble salt of a hydrated aromatic sulfonic acid containing several hydrocarbon residues as side chains.

9. A preparation for softening and oiling textile fibers comprising in emulsion, an oil, water, and alkylated cellulose, and a water-soluble aromatic sulfonic acid compound containing a hydrocarbon residue as side chain.

10. A preparation for softening and oiling textile fibers comprising in emulsion, an oil, water, an alkylated cellulose, and a water-soluble salt of an aromatic sulfonic acid containing a hydrocarbon residue as side chain.

11. A preparation for softening and oiling textile fibers comprising in emulsion, an oil, water, an alkylated cellulose, and an alkali metal salt of an aromatic sulfonic acid containing hydrocarbon residue as side chain.

12. A preparation for softening and oiling textile fibers comprising in emulsion, an oil, water, an alkylated cellulose, and a water-soluble aromatic sulfonic acid compound containing several hydrocarbon residues as side chains.

13. A preparation for softening and oiling textile fibers comprising in emulsion, an oil, water, an alkylated cellulose, and a water-soluble salt of an aromatic sulfonic acid containing several hydrocarbon residues as side chains.

14. A preparation for softening and oiling textile fibers comprising in emulsion, an oil, water, an alkylated cellulose, and an alkali metal salt of an aromatic sulfonic acid containing several hydrocarbon residues as side chains.

In testimony whereof, I affix my signature.

SIGISMUND FUCHS.